

1

3,135,606

**NOVEL PHOTOGRAPHIC PRODUCTS AND PROCESSES EMPLOYING ANTHRAQUINONE DYE**

Elkan R. Blout, Belmont, Marilyn R. Cohler, Brookline, Milton Green and Myron S. Simon, Newton Center, and Robert B. Woodward, Belmont, Mass., assignors to Polaroid Corporation, Cambridge, Mass., a corporation of Delaware

No Drawing. Filed Oct. 26, 1962, Ser. No. 233,461  
38 Claims. (Cl. 96—29)

This invention relates to photography and more particularly to products, compositions and processes for the development of photosensitive silver halide elements.

It is one object of the present invention to provide novel processes and compositions for the development of silver halide emulsions, in which novel colored developing agents are used to develop a latent image.

Another object is to provide novel processes and compositions for the development of silver halide emulsions, in which the novel developing agent is capable of developing a latent image and imparting a reversed or positive colored image of said latent image to a superposed image-receiving material.

A further object is to provide novel products, processes and compositions suitable for use in preparing monochromatic and multichromatic photographic images.

Other objects of the invention will in part be obvious and will in part appear hereinafter.

The invention accordingly comprises the processes involving the several steps and the relation and order of one or more of such steps with respect to each of the others, and the products and compositions possessing the features, properties and the relation of elements which are exemplified in the following detailed disclosure, and the scope of the application of which will be indicated in the claims.

The objects of this invention may be accomplished by the use of certain novel dyes which have the ability to develop latent images present in an exposed silver halide emulsion; thus they may be referred to as dye developers. These novel dyes or dye developers will be further described hereinafter.

The photographic processes and compositions disclosed herein are particularly useful in the treatment of a latent image present in a photosensitive element, such as an exposed silver halide emulsion whereby a positive dye image thereof may be imparted to another element, herein referred to as an image-carrying or image-receiving element.

U.S. Patent No. 2,983,606, issued May 9, 1961, to Howard G. Rogers, discloses diffusion transfer reversal processes wherein a photographic negative material, such as a photographic element comprising an exposed silver halide emulsion layer containing a latent image, is developed in the presence of a dye developer to impart to an image-receiving element a reversed or positive dye image of said latent image by permeating into said emulsion layer a suitable liquid processing composition and bringing said emulsion layer into superposed relationship with an appropriate image-receiving layer. The inventive concepts herein set forth provide novel dye developers for use in such processes.

In carrying out the process of this invention, a photosensitive element containing a silver halide emulsion is exposed and wetted with a liquid processing composition, for example by immersing, coating, spraying, flowing, etc., in the dark, and the photosensitive element superposed, prior to, during or after wetting, on an image-receiving element. In a preferred embodiment, the photosensitive element contains a layer of dye developer, and the liquid processing composition is applied to the photosensitive element in a uniform layer as the photosensitive

2

element is brought into superposed position with an image-receiving element. The liquid processing composition permeates the emulsion to provide a solution of dye developer substantially uniformly distributed therein. As

5 the latent image is developed, the oxidation product of the dye developer is immobilized or precipitated in situ with the developed silver, thereby providing an image-wise distribution of unoxidized dye developer dissolved in the liquid processing composition. This immobilization is apparently due, at least in part, to a change in the solubility characteristics of the dye developer upon oxidation, and especially as regards its solubility in alkaline solutions. It may also be due, in part, to a tanning effect on the emulsion by the oxidized developing agent.

10 At least part of this image-wise distribution of unoxidized dye developer is transferred, by imbibition, to a superposed image-receiving element, said transfer substantially excluding silver or oxidized dye developer. The latter element receives a depthwise diffusion, from the emulsion, of unoxidized dye developer, without appreciably disturbing the image-wise distribution thereof, to provide a reversed or positive, colored image of the negative image.

15 The image-receiving element may contain agents adapted to mordant or otherwise fix the diffused, unoxidized dye developer. Imbibition periods of approximately one minute have been found to give good results, but this contact period may be adjusted where necessary to compensate for variations in temperature or other conditions. The desired positive image is revealed by stripping the image-receiving element from the photosensitive element at the end of the imbibition period.

20 The dye developers of this invention may be utilized in the photosensitive element, for example, in, on or behind the silver halide emulsion, or they may be utilized in the image-receiving element or in the liquid processing composition. In a preferred embodiment, a coating or layer of the dye developer is placed behind the silver halide emulsion, i.e., on the side of the emulsion adapted to be located most distant from the photographed subject when the emulsion is exposed and preferably also adapted to be most distant from the image-receiving element when in superposed relationship therewith. Placing the dye developer behind the emulsion layer, as in the preferred embodiment, has the advantage of providing increased contrast in the positive image, and also minimizes any light-filtering action by the colored dye developer. In this preferred embodiment, the layer of dye developer may be applied by using a coating solution containing about 0.5 to 8%, by weight, of the dye developer. Similar concentrations may be used if the dye developer is utilized as a component of the liquid processing composition. In an especially useful mode of disposing the dye developers in the photosensitive elements, the dye developer is dissolved in a water-immiscible solvent and then dispersed in a gelatin coating solution. The coating solution is then applied to the photosensitive element, which is to be prepared, in the sequence desired.

25 The liquid processing composition which is used in the processes herein disclosed comprises at least an aqueous solution of an alkaline compound, for example, diethylamine, sodium hydroxide or sodium carbonate, and may contain the dye developer. In some instances, it may contain a conventional developing agent. If the liquid processing composition is to be applied to the emulsion by being spread thereon, preferably in a relatively thin, uniform layer, it may also include a viscosity-increasing compound constituting film-forming material of the type which, when spread over a water-absorbent base, will form a relatively firm and relatively stable film. A preferred film-forming material is a high molecular weight polymer such as a polymeric, water-soluble ether inert to



pared by the replacement of sulfo, halogen, nitro, hydroxyl, alkoxy or amino substituents on anthraquinone nuclei by amino groups derived from amines having the formula:



wherein Z and X have the same meaning as set forth above.

The 1 and 4 substituted anthraquinones such as those represented by Formulae 2 and 3 may be conveniently prepared from 1,4-diaminoanthraquinones and from 1,4-dihydroxyanthraquinones, i.e., quinizarins. When quinizarin is used in the preparation of the compounds, herein disclosed, the quinizarin may be first reduced to leuco quinizarin, then condensed, and the resulting product oxidized to the anthraquinone, by for example, aerial oxidation. When it is desired to prepare the dye developers herein disclosed directly from quinizarin it has been found that the reaction may be facilitated by carrying it out in the presence of an acid-acceptor and a mono-hydroxy-substituted aryl compound. As examples of monohydroxy-substituted aryl compounds, mention may be made of phenol, naphthol, cresol, xylol, etc. It has been further found that the condensation of quinizarin with the amine may also be facilitated by carrying the reaction out in the presence of an acid-acceptor and an ortho- or para-dihydroxy-substituted aryl compound. As examples of ortho- and para-dihydroxy-substituted aryl compounds, mention may be made of hydroquinone, catechol, naphthohydroquinone, and 1,2-dihydroxynaphthalene.

The dye developers within Formula 3 may be prepared by condensing an anthraquinone such as quinizarin with about an equivalent of an amine within Formula 4 and then with about an equivalent of an amine within formula:



wherein R is the same as above. It will be understood that the order of condensing the amines may be reversed to suit particular needs. It will be further understood that dye developers within Formula 2 wherein the  $-\text{NH}-\text{Z}-\text{X}$  radicals are different may be similarly prepared.

The compounds within the scope of this invention may be further prepared by condensing an amino-substituted anthraquinone with a haloalkyl-substituted benzenoid silver halide developer.

It should be noted that the process of this invention permits one to convert compounds which are not dyes into products which are both dyes and photographic developing agents.

In certain instances, in using the dye developers herein disclosed in photographic processes, it may be desirable to temporarily shift the light absorption characteristics of such dye developers so that they absorb less light of the higher wave lengths. One such instance when such a shift is desirable occurs when a cyan dye developer, such as the 1,4-diamino-substituted developers disclosed herein, are disposed in red-sensitive silver halide emulsions. In such a use it may be desirable that said dye developers absorb less red light until at least after exposure. In instances such as this and in other instances where such a shift is desirable, it has been found that the leuco-form of the anthraquinones may be employed. When it is desired to shift the color back, such as, for example, after exposure or transfer, such a shift may be made by a simple oxidation, e.g., aerial oxidation.

X has been defined as a benzenoid silver halide developing radical. Such benzenoid silver halide developers in general comprise an aryl nucleus which is substituted by at least two substituents selected from the group consisting of amino, alkylamino, and/or hydroxyl groups. The amino, alkylamino, and hydroxyl substituents are

usually substituted in ortho- or para-relationship with respect to each other, however, in polynuclear benzenoid developers they may be substituted in different rings. When substituted in different rings the positions which such substituents must occupy with respect to each other in order to provide a developing function are known from texts, such as, for example, The Theory of the Photographic Process, C. E. K. Mees, (revised edition, 1954), The Macmillan Co., New York, N.Y., p. 544 et seq. In a preferred embodiment of this invention the benzenoid silver halide developing radical is selected from those comprising dihydroxy-substituted benzene or naphthalene nuclei and more preferably comprises an ortho- or para-dihydroxybenzene radical. The para-dihydroxybenzenes have been found particularly useful. It should be noted that the radical X may contain substituents other than those which supply the silver halide developing function so long as such substituents do not adversely affect the silver halide developing ability; such substituents include alkyl, alkoxy, hydroxy, amino, halogen, etc.

Where the developing function possessed by X is supplied by hydroxyl or amino groups, it may be desirable to protect these groups, during synthesis, as by acylation, to avoid side reactions or oxidation. The protective groups are removed, as by hydrolysis, prior to photographic use.

As examples of dye developers within the scope of this invention, mention may be made of:

30



45 1,4-bis(α-methyl-β-hydroxyethylamino)-anthraquinone



60 1,4-bis(α-methyl-β-hydroxyethylamino)-5,8-dihydroxyanthraquinone



70 1-(α-hydroxymethyl-propylamino)-4-(α-methyl-β-hydroxyethylamino)-anthraquinone



1-( $\alpha$ -hydroxymethyl-propylamino)-4-( $\alpha$ -methyl- $\beta$ -hydroquinonyl-ethylamino)-5,8-dihydroxyanthraquinone

Other dye developers which have been prepared and are illustrative of the compounds within the scope of this invention include:

- 1-hydroxy-4-( $\alpha$ -methyl-hydroquinonyl-ethylamino)-anthraquinone.
- 1,4-bis-( $\gamma$ -hydroquinonyl- $\alpha$ -methyl-propylamino)-5,8-dihydroxyanthraquinone.
- 1,4-bis-( $\alpha$ -methyl- $\gamma$ -hydroquinonylpropylamino)-anthraquinone.
- 1,5-bis-hydroquinonylmethylamino-anthraquinone.
- 1,4-bis-hydroquinonylmethylamino-anthraquinone.
- 1,4-bis-( $\alpha$ -methyl- $\beta$ -hydroquinonyl-ethylamino)-6,7-dichloroanthraquinone.
- 1-( $\alpha$ -methyl- $\beta$ -hydroquinonyl-ethylamino)-4-( $\alpha$ -ethyl- $\beta$ -hydroquinonyl-ethylamino)-anthraquinone.
- 1-( $\alpha$ -methyl- $\beta$ -hydroquinonyl-ethylamino)-4-( $\alpha$ -ethyl- $\beta$ -hydroquinonyl-ethylamino)-5,8-dihydroxy-anthraquinone.
- 1,4-bis-( $\alpha$ -methyl-2',5'-dihydroxybenzylamino)-anthraquinone.
- 1,4-bis-( $\alpha$ -methyl- $\beta$ -hydroquinonyl-ethylamino)-5,8-bis-benzene-sulfonamido-anthraquinone.
- 1,4-bis-( $\alpha$ -methyl- $\beta$ -hydroquinonyl-ethylamino)-5-hydroxy-8-amino-anthraquinone.
- 1-( $\alpha$ -hydroxymethyl-propylamino)-4-( $\alpha$ -methyl- $\beta$ -hydroquinonyl-ethylamino)-5-hydroxyanthraquinone.
- 1,4-bis-( $\alpha$ -methyl- $\beta$ -hydroquinonyl-ethylamino)-5-hydroxyanthraquinone.
- 1,4-bis-( $\beta$ -hydroquinonyl-ethylamino)-anthraquinone.
- 1-[ $\beta$ -( $\beta$ -hydroquinonyl-ethyl)-phenylamino]-anthraquinone.
- 1-( $\alpha$ -hydroxymethyl-propylamino)-4-[ $\beta$ -(4'-methyl-2',5'-dihydroxyphenyl)- $\alpha$ -methyl-ethylamino]-anthraquinone.
- 1-ethylamino-4-[ $\beta$ -(3',4'-dihydroxyphenyl)-ethylamino]-anthraquinone.
- 1-chloro-4-( $\beta$ -hydroquinonyl-ethylamino)-anthraquinone.
- 1-hydroxy-4-[ $\beta$ -(3',4'-dihydroxyphenyl)-ethylamino]-anthraquinone.
- 1-chloro-5-( $\beta$ -hydroquinonyl-ethylamino)-anthraquinone.
- 1,4-bis-[ $\beta$ -(3',4'-dihydroxyphenyl)-ethylamino]-5,8-dihydroxyanthraquinone.
- 1,8-bis-[ $\beta$ -(3',4'-dihydroxyphenyl)-ethylamino]-anthraquinone.
- 1-[ $\beta$ -(3',4'-dihydroxyphenyl)-ethylamino]-anthraquinone.
- 1,5-bis-hydroquinonyl-ethylamino-anthraquinone.
- 1,5-bis-[ $\beta$ -(3',4'-dihydroxyphenyl)-ethylamino]-anthraquinone.
- 1,5-bis-( $\beta$ -hydroquinonyl-ethylamino)-anthraquinone.
- 1,8-bis-( $\beta$ -hydroquinonyl-ethylamino)-anthraquinone.
- 1-[ $\beta$ -(3',4'-dihydroxyphenyl)-ethylamino]-5-nitro-anthraquinone.
- 1,5-bis-( $\alpha$ -methyl- $\beta$ -hydroquinonyl-ethylamino)-anthraquinone.
- 1-( $\beta$ -hydroxyethylamino)-4-( $\beta$ -hydroquinonyl-ethylamino)-anthraquinone.
- 1,4-bis-[ $\beta$ -(3',4'-dihydroxyphenyl)-ethylamino]-anthraquinone.
- 1-( $\beta$ -hydroxyethylamino)-4-( $\alpha$ -methyl- $\beta$ -hydroquinonyl-ethylamino)-5,8-dihydroxyanthraquinone.

1,4-bis-( $\alpha$ -ethyl- $\beta$ -hydroquinonyl-ethylamino)-anthraquinone.

1-methylamino-4-( $\beta$ -hydroquinonyl-ethylamino)-anthraquinone.

5 1- $\beta$ -hydroxyethylamino-4-( $\alpha$ -methyl- $\beta$ -hydroquinonyl-ethylamino)-anthraquinone.

The following nonlimiting examples illustrate the preparation of dye developers within the scope of this invention.

10 *Example 1*

One mole of leucoquinizarin and four moles of 4-(beta-aminoethyl)-catechol hydrobromide are refluxed in butanol for four hours under nitrogen in the presence of four moles of sodium bicarbonate. The reaction mixture is then acidified with dilute hydrochloric acid (in the presence of sufficient methanol to maintain a single liquid phase) and filtered. The precipitate is oxidized by dissolving in pyridine open to the air and boiling until no further color change takes place. Crystallization from ethyl acetate-petroleum ether yields 1,4-bis-[ $\beta$ -(3',4'-dihydroxyphenyl)-ethylamino]-anthraquinone, melting at 159-161°C. This compound is soluble in acetone, ethyl alcohol, ethyl acetate and pyridine, and insoluble in water and petroleum ether. It is stable in neutral or acid solution, but unstable in base in the presence of air. Analysis of the product shows:

|                 | C    | H   | N   |
|-----------------|------|-----|-----|
| Calculated..... | 70.6 | 5.1 | 5.5 |
| Found.....      | 70.5 | 5.3 | 5.1 |

5 11 *Example 2*

35 Leucoquinizarin (1.2 g.; 0.005 mole), 2-beta-aminoethyl-hydroquinone hydrobromide (2.8 g.; 0.012 mole), and sodium bicarbonate (0.01 g.; 0.012 mole) are refluxed in 25 ml. of pyridine for two hours under nitrogen. One ml. of concentrated hydrochloric acid and one ml. of water are added to the reaction mixture and air is bubbled through at the reflux point until the color of the reaction mixture has gone to a clear blue without traces of green color. The reaction mixture is filtered into 150 ml. of 10% hydrochloric acid, the filtrate cooled in ice, and filtered. The solid is washed with water and ethyl acetate and then dissolved in ethanol and concentrated (under nitrogen) to give 0.5 g. (32% yield) of 1,4-bis-(beta-hydroquinonyl-ethylamino)-anthraquinone melting at 154-157°C. Concentration of the mother liquor gives an additional yield of 1.03 g. of product of lesser purity. The product in an ethanol solution is pure blue in color in daylight. It is slightly soluble in acetone and ethyl acetate, soluble in alcohol and pyridine but insoluble in water and petroleum ether. It is stable in neutral or acid solution, but unstable in base in the presence of air. Nitrogen analysis of the product shows a nitrogen value of 5.8% as compared with a calculated value of 5.5%.

60 It has been found that the yield of the desired 1,4-bis-[ $\beta$ -(2',5'-dihydroxyphenyl)-ethylamino]-anthraquinone may be increased, and its purification simplified, by increasing the reaction time, as illustrated by the following example:

65 *Example 3*

70 Leucoquinizarin (2.3 g.; 0.0097 mole), 2-(beta-aminoethyl)-hydroquinone hydrobromide (5 g.; 0.021 mole), and sodium bicarbonate (1.8 g.; 0.021 mole) are refluxed, under nitrogen, for 21 hours in 100 cc. of pyridine and 3 cc. of water. The reaction mixture is then cooled below the boiling point. A 1:1 concentrated hydrochloric acid and water mixture (4 cc.) is added. Air is bubbled through the mixture at the reflux point until the color of the mixture has gone to a clear blue without traces of a green color. The solution is cooled and then fil-

tered into excess 10% hydrochloric acid. The resulting precipitate is filtered, washed with water, and pulverized. The pulverized product is washed with hot alcohol to obtain 3 g. (60.3% yield) of the desired 1,4-bis-[beta-hydroquinonyl-ethylamino]-anthraquinone. The ethanol washings are precipitated with water and the precipitate washed with hot ethanol to obtain an additional 0.3 g. of the desired product.

Although hydrobromide salts of the



compounds have been used in the above examples, the free amine or other salts thereof, e.g., the hydrochloride, may be used.

*Example 4*

12 g. leucoquinizarin (0.05 mole), 32.2 g. sodium bicarbonate and 25 g. of 2-aminopropylhydroquinone-hydrobromide were placed in 375 cc. of nitrogen-deaerated pyridine and 10 cc. of water and refluxed overnight under vacuum. 8 cc. of a 50% hydrochloric acid solution were added and air was bubbled into the solution over a steam bath for about an hour until a blue solution resulted. The product was precipitated into dilute hydrochloric acid and purified twice from acetone into water. The resulting precipitate was further washed with a 5 to 10% acetone-water solution until the washings no longer showed a yellow-brown color. The product was heated with 300 cc. of ethyl acetate until most of it dissolved. The undissolved material was 1-(beta-hydroquinonyl-alpha-methyl-ethylamino)-4-hydroxy-anthraquinone. The ethyl acetate solution was concentrated under nitrogen to about 80 cc. and precipitated into hexane. The ethyl acetate-hexane purification was repeated and then followed with a crystallization from a (4 to 6 by volume) water-ethyleneglycol monomethyl ether solution. The 1,4-bis-(beta-hydroquinonyl-alpha-methyl-ethylamino)-anthraquinone produced sinters at 130 to 132° C. and a spectrographic analysis showed the following:

$$\epsilon 642 \text{ m}\mu=20,000$$

The following Example 5 provides an alternative method for preparing the compound of Example 4 using quinizarin.

*Example 5*

2.4 g. quinizarin (0.01 mole), 8.6 g. beta-amino-alpha-methyl-ethylhydroquinone-hydrobromide (0.035 mole), 0.34 g. sodium carbonate, 3.4 phenol (0.036 mole), 12 cc. 95% ethanol and 8 cc. of water were mixed together and deaerated with nitrogen. The mixture was then refluxed under nitrogen for 72 hours, then cooled and washed out of the reaction flask with a dilute hydrochloric acid solution into ice water. The resulting precipitate was filtered, washed several times with warm water and dissolved in acetone. The acetone solution was filtered and poured with rapid stirring into a large volume of an iced 2% hydrochloric acid solution. The resulting precipitate was warmed on a steam bath to 40° C. to aid coagulation, filtered while still warm and washed with water. The product was purified twice from acetone into hexane and dried under a heat lamp.

*Example 6*

5.5 g. of 5,8-benzenesulfonamide-quinizarin (0.01 mole), 9.95 g. of beta-amino-alpha-methyl-ethylhydroquinone-hydrobromide (0.04 mole), 1.8 g. of sodium carbonate, 3.4 g. of sodium bicarbonate and 3.75 g. phenol were placed in a deaerated flask, mixed with a nitrogen deaerated solution comprising 17 ml. of 95% ethanol and 11.5 ml. of water and reacted under nitrogen at a temperature of 105-7° C. for 101 hours. The reaction mixture was precipitated into a 2% hydrochloric acid solution filtered, and the resulting precipitate was redispersed in a 2% hydrochloric acid solution. The precipitate was then filtered and washed with a 2% hydrochloric acid solution

until the washings were colorless. The product was then precipitated from ethyleneglycol monomethyl ether to dilute hydrochloric acid, filtered and dried. The product was further purified by twice precipitating it from ethyl acetate into hexane. The 5,8-benzenesulfonamide-1,4-bis-(beta-hydroquinonyl-alpha-methyl-ethylamino)-anthraquinone produced sintered at 142° C., and, upon a spectrographic analysis in ethyleneglycol monomethyl ether, showed the following:

$$\begin{aligned} 10 & \epsilon 672 \text{ m}\mu=19,200 \\ & \epsilon 622 \text{ m}\mu=14,000 \\ & \epsilon 580 \text{ m}\mu=11,600 \end{aligned}$$

*Example 7*

15 2.3 g. of leuco-1,4,5,8-tetrahydroxyanthraquinone, 5.6 g. of 2-aminopropyl-hydroquinone hydrobromide and 1.9 g. sodium bicarbonate were dissolved in 50 ml. of pyridine and 2 ml. of water and refluxed for 64 hours. The solution was aerated at its boiling point for 1.2 hours and 20 then allowed to stand at room temperature for an additional 18 hours. The product was precipitated into a 10% hydrochloric acid solution and taken up in 300 ml. of methanol. The methanol solution was evaporated until crystallization began and then it was allowed to stand 25 overnight. The 1,4-bis-(beta-hydroquinonyl-alpha-methyl-ethylamino)-5,8-dihydroxyanthraquinone produced had a melting point of 224° C. and upon a spectrographic analysis showed the following:

$$\begin{aligned} 30 & \epsilon 620 \text{ m}\mu=20,600 \\ & \epsilon 675 \text{ m}\mu=30,000 \end{aligned}$$

*Example 8*

35 36.0 g. quinizarin (0.15 mole) and 50 g. phenol were added to 180 ml. of ethanol and 120 ml. of water and deaerated with nitrogen. 5 g. of sodium carbonate and 13.4 g. of 2-amino-1-butanol (0.15 mole) were added and the mixture was refluxed for 40 minutes under nitrogen. 37.2 g. of 2-aminopropylhydroquinone-hydrobromide (0.15 mole) and 12.6 g. sodium bicarbonate were then 40 added and refluxing was continued under nitrogen for another 22 hours until the reaction was completed. The reaction mixture was poured into 10% hydrochloric acid yielding a gummy mass. The gummy mass was purified twice from acetone into dilute hydrochloric acid and then 45 from ethyleneglycol monoethyl ether into dilute hydrochloric acid. The mass was further purified twice from ethylacetate into hexane and dried in a vacuum desiccator. The 1-(alpha-hydroxymethyl-propylamino)-4-(beta-hydroquinonyl-alpha-methyl-ethylamino)-anthraquinone obtained 50 showed the following in a spectrograph analysis:

$$\begin{aligned} & \epsilon 640 \text{ m}\mu=19,000 \\ & \epsilon 594 \text{ m}\mu=16,400 \\ & \epsilon 558 \text{ m}\mu=8,800 \end{aligned}$$

*Example 9*

55 13.7 g. of leuco-1,4,5,8-tetrahydroxyanthraquinone (0.05 mole), 12.4 g. of 2-aminopropylhydroquinone-hydrobromide (0.05 mole) and 4.2 g. of sodium bicarbonate (0.05 mole) were added to 150 ml. of pyridine and refluxed for 24 hours under nitrogen. 5.0 g. of 2-amino-butanol (0.056 mole) were added and the refluxing was 60 continued another 24 hours under nitrogen. 5 cc. of concentrated hydrochloric acid was added and air was 65 bubbled through the solution at 70-85° C. for about 24 hours. The mixture was cooled and added to a solution comprising 3000 ml. of water and 250 ml. of concentrated hydrochloric acid. The resulting precipitate was filtered off and washed with cold water until the filtrate was 70 colorless. The solid was vacuum dried, powdered and mixed with 1 to 2 volumes of celite and extracted with 200-300 ml. of ethyl acetate in a Soxhlet extractor until the extract was nearly colorless. Upon cooling, the extract was stirred into about 2500 ml. of hexane and the 75 resulting precipitate was filtered and dried. The 1-(alpha-

## 11

hydroxymethyl-propylamino) - 4 - ( $\beta$  - hydroquinonyl- $\alpha$ -methyl-ethylamino) - 5,8 - dihydroxyanthraquinone produced, showed, upon a spectrographic analysis, the following:

$$\epsilon 675 \text{ m}\mu = 28,000$$

## Example 10

2.56 g. of 1,4,5-trihydroxy-anthraquinone (0.01 mole), 8.6 g. of 2 - aminopropylhydroquinone - hydrobromide (0.036 mole), 0.34 g. of sodium carbonate, 2.9 g. sodium bicarbonate (0.36 mole) and 3.4 g. of phenol were added to 15 ml. of water and 20 ml. of ethanol and refluxed under nitrogen for 49 hours. The reaction mixture was poured into a 15% hydrochloric acid solution and the resulting precipitate was filtered and washed several times with water. To insure the absence of leuco material the precipitate was dissolved in boiling pyridine in air, then precipitated into dilute hydrochloric acid. The resulting gummy solid was precipitated from acetone into hexane and dissolved in methyl acetate. The methyl acetate solution was concentrated and, on cooling, the product crystallized out in microneedles. The product was filtered, washed several times with methyl acetate containing enough hexane to prevent solubilization, and dried at room temperature overnight. The 5-hydroxy-1,4-bis-( $\beta$ -hydroquinonyl- $\alpha$ -methyl-ethylamino) - anthraquinone produced melted at 150-6° C. and showed the following in a spectrographic analysis using ethylene-glycol monomethyl ether as the solvent:

$$\begin{aligned} \epsilon 655 \text{ m}\mu &= 26,600 \\ \epsilon 604 \text{ m}\mu &= 19,200 \end{aligned}$$

## Example 11

The procedure of Example 6 was followed except that 3.09 g. of 6,7-dichloroquinizarin (0.01 mole) was used in place of the 5,8-benzene-sulfonamidoquinizarin. After reacting at reflux for 100 hours the reaction mixture was cooled and added to 160 ml. of 10% hydrochloric acid to precipitate the product. The product was purified once from acetone into dilute hydrochloric acid and a second time from warm acetone into hexane. The 1,4-bis-( $\beta$ -hydroquinonyl -  $\alpha$  - methyl-ethylamino) - 6,7 - dichloroanthraquinone produced, upon spectrographic analysis, showed the following:

$$\epsilon 657 \text{ m}\mu = 21,400$$

An elemental nitrogen analysis showed the following:

| Calculated | Percent |
|------------|---------|
| 4.63       | 50      |
| 4.4        |         |

## Example 12

1.4 g. of 1,8-dichloroanthraquinone, 5.9 g.  $\beta$ -aminoethylhydroquinone-hydrobromide and 2.1 g. sodium bicarbonate were added to 15 cc. of quinoline and refluxed for 4½ hours under nitrogen. The reaction mixture was added to dilute hydrochloric acid and ice, filtered and washed with dilute hydrochloric acid. The precipitate was dissolved in ethyl alcohol under nitrogen, and the resulting ethyl alcohol solution was filtered and concentrated under nitrogen. The resulting crystalline product was filtered and washed with a small amount of cold ethanol. The product was still further purified by crystallization from ethanol under nitrogen. The resulting 1,8-bis-( $\beta$ -hydroquinonyl-ethylamino) - anthraquinone sintered at 163-8° C. and upon a spectrographic analysis, using dimethyl formamide as the solvent, showed the following:

$$\epsilon 545 \text{ m}\mu = 7,500$$

## Example 13

1.2 g. of 1,5-dichloroanthraquinone, 6.0 g.  $\beta$ -aminoethylhydroquinone and 5.8 g. of sodium bicarbonate were added to 130 cc. of quinoline and reacted at reflux for three hours. The quinoline was removed under vacuum

## 12

and ethyl alcohol was added. Ethyl ether was then added and the resulting white precipitate was filtered. The filtrate was concentrated under vacuum and taken up in acetone from which it was precipitated into petroleum ether. The gummy product was precipitated twice from ethyl alcohol, once into dilute hydrochloric acid and once into water. The 1,5-bis-( $\beta$ -hydroquinonyl-ethylamino) - anthraquinone melts at 135 to 145° C. and upon a spectrographic analysis shows the following:

$$\epsilon 518-527 \text{ m}\mu = 11,200$$

## Example 14

1.99 g. of 1,5-dihydroxy-4,8-diaminoanthraquinone, 7.45 g.  $\beta$  - hydroquinonyl- $\alpha$ -methyl-ethylamine-hydrobromide, 2.3 g. of sodium bicarbonate and 1 g. zinc dust were placed in 15 ml. of butanol and refluxed under nitrogen for about 20 hours. The reaction mixture was filtered and poured into dilute hydrochloric acid. The resulting sludge was precipitated twice from ethylene-glycol monomethyl ether into saturated brine, dried very carefully and precipitated twice from ethyl acetate into hexane. The product was chromatographed on aluminum sulfate, eluted first with benzene and then with ethyl acetate and evaporated to dryness. The dry product was once again precipitated from ethyl acetate into hexane and dried. A spectrographic analysis of the 1,4-bis-( $\beta$ -hydroquinonyl -  $\alpha$  - methyl-ethylamino) - 5 - hydroxy-8-amino-anthraquinone showed the following:

$$\epsilon 675 \text{ m}\mu = 21,400$$

The spectrum of the product obtained would indicate that it still was not completely purified.

## Example 15

2.5 g. of 1-nitro-anthraquinone and 10 g. of  $\beta$ -(*p*-amino-phenyl) - ethylhydroquinone - O,O - diacetate-hydrochloride were dissolved in 50 ml. of ethylene-glycol monomethyl ether and refluxed for 24 hours. The reactive mixture was filtered and precipitated into 1.5% hydrochloric acid. The tarry product was purified twice from ethylene-glycol monomethyl ether into an aqueous sodium chloride-sodium acetate solution. The precipitate was taken up in ethanol and water, deaerated with nitrogen and hydrolyzed with dilute sodium hydroxide on a steam bath for about two minutes. The product was precipitated with hydrochloric acid and purified once again from ethylene-glycol monomethyl ether into an aqueous sodium chloride-sodium acetate solution. A spectrographic analysis of the 1 - [*p* - (2',5' - dihydroxyphenethyl) - phenylamino]-anthraquinone showed the following:

$$\epsilon_{\text{max.}} = 6,400 \text{ at } 503 \text{ m}\mu$$

## Example 16

12.0 g. of quinizarin, 13 g. of 2-aminopropylhydroquinone-hydrobromide, 4.2 g. sodium bicarbonate, 1.7 g. of sodium carbonate and 17 g. of phenol were placed in 60 ml. of ethanol and 40 ml. of water and refluxed under nitrogen for 22 hours. Then 13.1 g. of 2-aminobutylhydroquinone-hydrobromide and 4.2 g. of sodium bicarbonate were added and the reaction mixture was refluxed for another 24 hours under nitrogen. The reaction mixture was precipitated into dilute hydrochloric acid and twice purified from ethylene-glycol monomethyl ether into saturated brine. The product was thoroughly dried and precipitated twice from ethyl acetate into hexane. A spectrographic analysis of the 1-( $\beta$ -hydroquinonyl- $\alpha$ -methyl-ethylamino) - 4 - ( $\gamma$  - hydroquinonyl -  $\alpha$  - methyl-propylamino)-anthraquinone produced showed the following:

$$\epsilon_{\text{max.}} = 16,000 \text{ at } 642 \text{ m}\mu$$

## Example 17

9.6 g. of quinizarin, 3.5 g. of 2-aminobutanol, 1.57 g. of sodium carbonate and 15.04 g. phenol were placed in 48 cc. of 95% ethanol and 32 cc. of water and refluxed

## 13

for 30 minutes. 10.48 g. of O-(4-methyl-2,5-dihydroxy-phenyl)- $\alpha$ -methyl-ethylamine-hydrobromide and 3.36 g. of sodium bicarbonate were then added and refluxing was continued for 18 hours. The resulting product was precipitated into a 10% hydrochloric acid solution and washed first with dilute hydrochloric acid and then with water. The precipitate was taken up in dimethylformamide, precipitated into dilute hydrochloric acid, washed with hot water and dried in a vacuum desiccator to yield a product which melted at 131 to 152° C. The product was further purified by precipitation from ethyl acetate into hexane, filtration through activated alumina, using ethanol as an eluant, and by precipitation once again from ethyl acetate into hexane. A spectrographic analysis of the 1 - ( $\alpha$  - hydroxymethyl - propylamino) - 4 - [ $\beta$  - (4'-methyl - 2',5' - dihydroxyphenyl) -  $\alpha$  - methyl - ethylamino]-anthraquinone produced showed the following:

$\epsilon_{642} \text{ m}\mu = 18,000$

An example of a photographic use of the dye developers herein disclosed, and set forth by way of illustration only, is the following:

## Example 18

A photosensitive element is prepared by coating a sub-coated cellulose acetate film base with a 4% aqueous gelatin solution followed by coating with a solution comprising:

|                                                                               |    |     |
|-------------------------------------------------------------------------------|----|-----|
| Cellulose acetate hydrogen phthalate                                          | g  | 4   |
| Acetone                                                                       | cc | 80  |
| Methanol                                                                      | cc | 20  |
| 1,4 - bis - [ $\beta$ - (3',4' - dihydroxyphenyl) - ethylamino]-anthraquinone | g  | 3.5 |

After this coating has dried, a silver iodobromide emulsion is applied. A liquid processing composition is prepared comprising:

|                                |    |     |
|--------------------------------|----|-----|
| Water                          | cc | 100 |
| Sodium carboxymethyl cellulose | g  | 4.5 |
| Sodium hydroxide               | g  | 1.5 |
| Metol                          | g  | 0.1 |

An image-receiving sheet is prepared by coating a polyvinyl butyral-coated baryta paper with a solution comprising:

|                                             |    |    |
|---------------------------------------------|----|----|
| N-methoxymethyl polyhexamethylene adipamide | g  | 4  |
| Isopropanol                                 | cc | 80 |
| Water                                       | cc | 20 |

The photosensitive element is exposed and the liquid processing composition is spread between the photosensitive element and the image-receiving element as these elements are brought into superposed relationship. After an imbibition period of one minute, the image-receiving element is separated and contains a cyan, positive dye image of the photographed subject.

## Example 19

A photosensitive element is prepared by coating a sub-coated cellulose acetate film base with a 4% aqueous gelatin solution followed by coating with a solution comprising:

|                                                                 |    |     |
|-----------------------------------------------------------------|----|-----|
| Cellulose acetate hydrogen phthalate                            | g  | 4   |
| Methyl Cellosolve                                               | cc | 100 |
| 1,4 - bis - (beta - hydroquinonyl - ethylamino) - anthraquinone | g  | 2.5 |

A liquid processing composition is prepared comprising:

|                                |    |     |
|--------------------------------|----|-----|
| Water                          | cc | 100 |
| Sodium carboxymethyl cellulose | g  | 4.0 |
| Sodium hydroxide               | g  | 2.0 |
| Metol                          | g  | 0.1 |

The photosensitive element is exposed and the liquid processing composition spread between the photosensitive ele-

## 14

ment and an image-receiving element, prepared as described in Example 18, as these elements are brought into superposed relationship. After an imbibition period of approximately one minute, the image-receiving element is separated and contains a cyan positive dye image of the photographed subject.

## Example 20

A photosensitive element is prepared as described in Example 18, using 2 g. of 1-chloro-4-(beta-hydroquinonyl-ethylamino)-anthraquinone in lieu of the dye developer set forth in that example. A liquid processing composition is prepared comprising:

|                                |    |     |
|--------------------------------|----|-----|
| Water                          | cc | 100 |
| Sodium hydroxide               | g  | 2.0 |
| Metol                          | g  | 0.1 |
| Ascorbic acid                  | g  | 0.2 |
| Sodium carboxymethyl cellulose | g  | 4.5 |

The photosensitive element is exposed and then brought into superposed relationship with an image-receiving element as the liquid processing composition is spread between said elements. The image-receiving element is prepared by applying a polyvinyl butyral coating to a cellulose acetate-coated baryta paper followed by a coating of a solution comprising:

|                                             |    |    |
|---------------------------------------------|----|----|
| N-methoxymethyl polyhexamethylene adipamide | g  | 4  |
| Ethanol                                     | cc | 85 |
| Furfuryl alcohol                            | cc | 15 |

After an imbibition period of approximately one minute, the image-receiving element is separated and contains a pink, positive dye image of the photographed subject.

## Example 21

A photosensitive element was prepared by coating a gelatin-subcoated cellulose acetate film base with a 1 to 1 methanolacetone solution comprising 3% of 1,4-bis-( $\alpha$ -methyl -  $\beta$  - hydroquinonyl-ethylamino) - 5,8 - dihydroxy-anthraquinone and 4% of cellulose acetate hydrogen phthalate. After this coating was dried, a silver iodobromide emulsion was applied. The film was exposed and an aqueous processing solution:

|                                |    |     |
|--------------------------------|----|-----|
| Sodium carboxymethyl cellulose | cc | 4.5 |
| Potassium bromide              | cc | 0.2 |
| Sodium hydroxide               | cc | 2.0 |
| 1-phenyl-3-pyrazolidone        | cc | 0.2 |

was spread between the photosensitive element and a nylon, image-receiving element such as used in Example 18. After an imbibition period of one minute, the image-receiving element was separated and contained a cyan image.

## Example 22

A photosensitive element was prepared by coating a gelatin-subcoated film base with an acetone-methanol solution (4 to 1 by volume) comprising 3% of 1,4-bis-( $\alpha$ -methyl -  $\beta$ -hydroquinonyl-ethylamino)-anthraquinone dye developer, as prepared in Example 4, and 4% of cellulose acetate hydrogen phthalate. A silver iodobromide emulsion was applied and the resulting element was exposed and processed in a manner similar to that employed in Example 21, except using 2.5% sodium hydroxide to produce a cyan transfer image.

## Example 23

A gelatin-subcoated film support was coated first with a tetrahydrofuran solution comprising 3% of 1- $\beta$ -hydroquinonyl-ethylamino-anthraquinone and 4% of cellulose acetate hydrogen phthalate and then with an iodobromide emulsion. Upon exposing and processing, in a manner similar to that employed in Example 18, except using 4% sodium hydroxide, a salmon-pink image was obtained.

## Example 24

A gelatin-subcoated film support was coated first with an acetone-methanol solution (4 to 1 by volume) comprising 3% of 1,5-bis-( $\beta$ -hydroquinonyl-ethylamino)-anthraquinone as prepared in Example 13, and 4% of cellulose acetate hydrogen phthalate and then with an iodobromide emulsion. Upon processing, using an image-receiving element having a polyvinyl alcohol image-receiving layer and an aqueous solution comprising:

|                                | Percent |
|--------------------------------|---------|
| Sodium carboxymethyl cellulose | 4.5     |
| Sodium hydroxide               | 2.0     |
| Potassium bromide              | 0.2     |
| Sodium carbonate               | 2.0     |
| N-methyl-p-aminophenol sulfate | 0.2     |

as the processing composition, a magenta image was obtained.

## Example 25

A gelatin-subcoated film support was coated first with an acetone-methanol solution (4 to 1 by volume) comprising 3% of 1,5-bis-[ $\beta$ -(3',4'-dihydroxyphenyl)-ethylamino]-anthraquinone and 4% of cellulose acetate hydrogen phthalate and then with an iodobromide emulsion. Upon processing, in a manner similar to that employed in Example 21, except that the processing solution also comprised 10% of urea, a magenta-transfer image was obtained.

## Example 26

A gelatin-subcoated film support was coated first with an acetone-methanol (4 to 1 by volume) solution comprising 3% of 1-[ $\beta$ -(3',4'-dihydroxyphenyl)-ethylamino]-5-nitroanthraquinone and 4% of cellulose acetate hydrogen phthalate and then with an iodobromide emulsion. Upon processing, in a manner similar to that employed in Example 21, a purple-magenta transfer image is obtained.

## Example 27

A photosensitive element was prepared by coating a gelatin-subcoated film support first with a 1 to 1 acetone-tetrahydrofuran coating solution comprising 4% of 1,5-bis-( $\alpha$ -methyl- $\beta$ -hydroquinonyl-ethylamino)-anthraquinone and 4% of cellulose acetate hydrogen phthalate and then with a silver iodobromide emulsion. Upon processing, in a manner similar to that employed in Example 21, using a polyvinyl alcohol-receiving sheet, a magenta image was obtained.

## Example 28

A gelatin-subcoated film support was first coated with an acetone-tetrahydrofuran coating solution (1 to 1 by volume) comprising 3% of 1- $\beta$ -hydroxyethylamino-4- $\beta$ -hydroquinonyl-ethylamino-anthraquinone and 4% cellulose acetate hydrogen phthalate and then with a silver iodobromide emulsion. Upon exposing and processing, in a manner similar to that employed in Example 21, except using an aqueous processing solution comprising:

|                                | Percent |
|--------------------------------|---------|
| Sodium carboxymethyl cellulose | 4.5     |
| 1-phenyl-3-pyrazolidone        | 0.2     |
| Sodium hydroxide               | 2.5     |
| Potassium bromide              | 0.2     |
| Ascorbic acid                  | 1.0     |

a cyan transfer image is obtained.

## Example 29

A photosensitive element was prepared, as in Example 28, except that 3% of 1-methylamino-4- $\beta$ -hydroquinonyl-ethylamino-anthraquinone was used in place of the 1- $\beta$ -hydroxyethylamino-4- $\beta$ -hydroquinonyl-ethylamino-anthraquinone. Upon exposing and processing, in a manner similar to that in Example 21, a cyan image was obtained.

## Example 30

An acetone-tetrahydrofuran coating solution (1 to 1 by volume) comprising 2% of cellulose acetate hydrogen phthalate and 5.5% of 1,4-bis-( $\alpha$ -methyl- $\beta$ -hydroquinonyl-ethylamino)-5,8-bis-benzene-sulfonamido-anthraquinone, as prepared in Example 6, was coated on a gelatin-subcoated cellulose acetate support. When the coating had dried, a coating of an iodobromide emulsion was applied. The above photosensitive element was exposed and then processed by spreading an aqueous processing solution comprising:

|                                   | Percent |
|-----------------------------------|---------|
| Sodium carboxymethyl cellulose    | 4.5     |
| Sodium hydroxide                  | 2.5     |
| 15 1-phenyl-3-pyrazolidone        | 1.0     |
| 2,5-bis-ethyleneiminohydroquinone | 0.45    |
| 6-nitrobenzimidazole              | 0.26    |

between said photosensitive element and a nylon image-receiving element, as prepared in Example 18. After an imbibition period of approximately one minute, the image-receiving element was separated and contained a dense blue image of the photographed subject.

## Example 31

A photosensitive element, similar to that of Example 30, was prepared using 5.0% of 1-( $\alpha$ -hydroxymethyl-propylamino)-4-( $\alpha$ -methyl- $\beta$ -hydroquinonyl-ethylamino)-anthraquinone, as prepared in Example 8, as the dye developer. Upon processing, in a manner similar to that used in Example 30, using a processing solution comprising:

|                                   | Percent |
|-----------------------------------|---------|
| Sodium hydroxide                  | 1.5     |
| Sodium carboxymethyl cellulose    | 4.5     |
| 1-phenyl-3-pyrazolidone           | 1.2     |
| 2,5-bis-ethyleneiminohydroquinone | 0.925   |
| 6-nitrobenzimidazole              | 0.12    |

a cyan positive image of the photographed subject was obtained.

## Example 32

A photosensitive element, similar to that of Example 30, was prepared using 4% of 1,4-bis-( $\alpha$ -methyl- $\beta$ -hydroquinonyl-ethylamino)-5,8-dihydroxyanthraquinone, as prepared in Example 7, as the dye developer. Upon developing in a manner similar to that used in Example 30, using a processing solution comprising:

|                                | Percent |
|--------------------------------|---------|
| Sodium hydroxide               | 1.5     |
| Sodium carboxymethyl cellulose | 4.5     |
| 1-phenyl-3-pyrazolidone        | 0.7     |
| Tertiary-butyl hydroquinone    | 0.3     |
| 6-nitrobenzimidazole           | 0.126   |

a cyan positive image was obtained.

## Example 33

A photosensitive element, similar to that of Example 30, was prepared using 5.5% of 1,4-bis-( $\alpha$ -methyl- $\beta$ -hydroquinonyl-ethylamino)-5-hydroxy-8-amino-anthraquinone as the dye developer. Upon processing, in a manner similar to that used in Example 30, using a processing solution comprising:

|                                   | Percent |
|-----------------------------------|---------|
| Sodium hydroxide                  | 2.0     |
| Sodium carboxymethyl cellulose    | 4.5     |
| 1-phenyl-3-pyrazolidone           | 0.6     |
| 2,5-bis-ethyleneiminohydroquinone | 0.4     |
| 6-nitrobenzimidazole              | 0.12    |

a cyan positive image was obtained.

## Example 34

A photosensitive element, similar to that of Example 30, was prepared using 5% of 1-( $\alpha$ -hydroxymethyl-propylamino)-4-( $\alpha$ -methyl- $\beta$ -hydroquinonyl-ethylamino) 5,8-

dihydroxyanthraquinone, 0.07% of 6-nitrobenzimidazole and 2% of Resoflex R-296 (a plasticizer, produced by Cambridge Industries, Cambridge, Mass.), in the coating solution. Upon processing, in a manner similar to that employed in Example 33, a cyan positive image of the photographed subject was obtained.

*Example 35*

A photosensitive element, similar to that of Example 34, was prepared using 5.5% of 1,4-bis-( $\alpha$ -methyl- $\beta$ -hydroquinonylethylamino)-6,7-dichloroanthraquinone, 0.4% of 6-nitrobenzimidazole and 0.4% of Resoflex R-296 in the coating solution. Upon developing, in a manner similar to that employed in Example 32, except reducing the 6-nitrobenzimidazole in the processing solution to 0.08%, a cyan positive image was obtained.

*Example 36*

A photosensitive element, similar to that of Example 30, was prepared using the 1-( $\alpha$ -hydroxymethyl-propylamino)-4-[ $\beta$ -(4'-methyl-2',5'-dihydroxyphenyl)- $\alpha$ -methyl-ethylamino]-anthraquinone as prepared in Example 17 as the developer. Upon developing in a manner similar to that employed in Example 30, a cyan positive image of the photographed subject was obtained.

The following example illustrates an embodiment of this invention wherein the leuco-form of the dye developer is used in a photosensitive element.

*Example 37*

A photosensitive element was made up similar to that in Example 21, using 3% of 1,4-bis-( $\beta$ -hydroquinonyl-ethylamino)-leucoanthraquinone. Upon processing, in a manner similar to that employed in Example 21, and after allowing time for aerial oxidation, a cyan image was obtained.

The dye developers of this invention are also useful in integral multilayer photosensitive elements for use in multicolor diffusion transfer processes. As an example of such photosensitive elements, mention may be made of the photosensitive elements disclosed and claimed in the co-pending U.S. application of Edwin H. Land and Howard G. Rogers, Serial No. 565,135, filed February 13, 1956, wherein at least two selectively sensitized photosensitive strata are superposed on a single support and are processed, simultaneously and without separation, with a single common image-receiving element. A suitable arrangement of this type comprises a support carrying a red-sensitive silver halide emulsion stratum, a green-sensitive silver halide emulsion stratum and a blue-sensitive silver halide emulsion stratum, said emulsions having associated therewith, respectively, a cyan dye developer, a magenta dye developer and a yellow dye developer. In one of the preferred embodiments of photosensitive elements of this type, the dye developers are disposed in separate alkaline permeable layers behind the photosensitive silver halide emulsion stratum with which they are associated.

The photosensitive elements within the scope of this invention may be used in roll film units which contain a plurality of photosensitive frames. The photosensitive elements of this invention are especially useful in composite roll film intended for use in a "Polaroid Land Camera," sold by Polaroid Corporation, Cambridge 39, Massachusetts, or a similar camera structure such, for example, as the camera forming the subject matter of U.S. Patent No. 2,435,717, issued to Edwin H. Land on February 10, 1948. In general, such composite roll films comprise a photosensitive roll, a roll of image-receiving material and a plurality of pods containing an aqueous alkaline processing solution. The rolls and pods are so associated with each other that, upon processing, the photosensitive element may be superposed on the image-receiving element and the pods may be ruptured to spread the aqueous alkaline processing solution between the superposed elements. The nature and construction of the pods used in such units are well known to the art. See, for example, U.S. Patent

Nos. 2,543,181 and 2,634,886, issued to Edwin H. Land.

It should be noted that certain dye developers within the scope of this invention may be subject to color changes as a result of pH changes in the portion of the image-receiving element to which they are diffused. Since the dye developer is generally rendered effective by solution in an aqueous alkaline liquid processing composition, it accordingly is necessary to assure that the environment in which the transferred and unreacted dye developer is deposited has, or is capable of attaining, the requisite pH value affording the desired color to the diffused dye developer. This may be accomplished by use of a volatile basic compound, such as diethylamine, in the liquid processing composition. If sodium hydroxide is utilized in the processing liquid, it becomes carbonated after processing and by contact with the air, and this is effective to provide the desired pH change. Further control of the pH of the transferred and unreacted dye developer may be had by utilizing an image-receiving element which is difficultly penetrable by alkali, for example an appropriate nylon such as N-methoxymethyl polyhexamethylene adipamide, or by the use of an image-receiving element in which an acid or an acid-forming compound, for example oleic acid, has been incorporated.

It will be noted that the liquid processing composition may, and in the above examples does, contain one or more conventional developers, such as Metol, ascorbic acid, hydroquinones, 3-pyrazolidones, e.g., 1-phenyl-3-pyrazolidone (Phenidone), and 1-phenyl-4,4-dimethyl-3-pyrazolidone. Although the dye developers in and of themselves can carry out the development, the conventional developers serve to accelerate and possibly initiate the action of the dye developer. In certain instances, it is believed that the oxidation of the dye developers may involve a cross oxidation with the oxidized conventional developers.

The dye developers of this invention may be used also in conventional photographic processes, such as tray or tank development of conventional photosensitive films, plates or papers to obtain black and white, monochromatic or toned prints or negatives. By way of example, a developer composition suitable for such use may comprise an aqueous solution of approximately 1-2% of the dye developer, 1% sodium hydroxide, 2% sodium sulfite and 0.05% potassium bromide. After development is completed, any unreacted dye developer is washed out of the photosensitive element, preferably with an alkaline washing medium or other medium in which the unreacted dye is soluble. The expression "toned" is used to designate photographic images wherein the silver is retained with the precipitated dye, whereas "monochromatic" is intended to designate dye images free of silver.

It should be noted that the dye developers of this medium are self-sufficient to provide the desired color image and do not depend upon coupling reactions to produce the desired color. They thus provide a complete departure from conventional photographic color processes in which the color is produced by a coupling reaction between a "color former" or "coupler" and the oxidized developing agent, as well as so-called auto-coupling processes in which color is obtained by a reaction of the oxidized developing agent with unoxidized developing agent.

It will be apparent that, by appropriate selection of the image-receiving element from among suitable known opaque and transparent materials, it is possible to obtain either a colored positive reflection print or a colored positive transparency. Likewise, the inventive concepts herein set forth are adaptable for multicolor work by the use of special photographic materials, for example, film materials of the type containing two or more photosensitized elements associated with an appropriate number of image-receiving elements and adapted to be treated with one or more liquid processing compositions, appropriate dye developers suitable to impart the desired subtractive

colors being incorporated in the photosensitized elements or in the liquid processing compositions. Examples of such photographic materials are disclosed in U.S. Patent No. 2,647,049 to Edwin H. Land.

As set forth above, the dye developers of this invention wherein Z is lower alkylene unexpectedly provide a substantial increase in the density of the transfer images as compared with images produced, under similar conditions, using the dye developers disclosed in the above-mentioned application Serial No. 449,514 (now abandoned), wherein the Z group is absent. The following chart is illustrative of this increase in density and gives a comparison under substantially similar test conditions between some of the dye developers of this invention and 1,4-bis-(2',5'-dihydroxyanilino)-anthraquinone, one of the dye developers disclosed in application Serial No. 449,514 wherein the Z group is absent.

| Compound                                                                                                  | D <sub>max</sub> | D <sub>min</sub> | Δ    |
|-----------------------------------------------------------------------------------------------------------|------------------|------------------|------|
| (a) 1,4-bis-(2',5'-dihydroxyanilino)-anthraquinone                                                        | 0.64             | 0.1              | 0.54 |
| (b) 1,4-bis-( $\beta$ -hydroquinonyl-ethylamino)-anthraquinone (Example 2)                                | 1.14             | 0.24             | 0.90 |
| (c) 1,4-bis-( $\beta$ -hydroquinonyl- $\alpha$ -methyl-ethylamino)-anthraquinone (Example 4)              | 1.48             | 0.04             | 1.44 |
| (d) 1,4-bis-( $\beta$ -hydroquinonyl- $\alpha$ -methyl-ethylamino)-5,8-dihydroxyanthraquinone (Example 7) | 1.64             | 0.05             | 1.59 |

The inventive concepts herein set forth are adaptable for the formation of colored images in accordance with the photographic products and processes described and claimed in the copending application of Edwin H. Land, Serial No. 448,441, filed August 9, 1954, now U.S. Patent No. 2,968,554, issued January 17, 1961.

The novel compounds herein disclosed are also suitable for use as dyes for textile fibres.

In the preceding portions of the specification the expression "Color" has been frequently used. This expression is intended to include the use of a plurality of colors to obtain black.

The present application is concerned with the photographic products, processes and compositions and is a continuation in part of application Serial No. 824,785, filed July 3, 1959 (now abandoned), which in turn is a continuation in part of application Serial No. 478,922, filed December 30, 1954, now abandoned.

Since certain changes may be made in the above products, compositions and processes without departing from the scope of the invention herein involved, it is intended that all matter contained in the above description shall be interpreted as illustrative and not in a limiting sense.

What is claimed is:

1. In a process of forming a photographic image in color, the steps which comprise developing an exposed silver halide emulsion with an aqueous alkaline solution containing a dye developer having an anthraquinone nucleus, at least one and not more than two of the nuclear carbon atoms of said anthraquinone nucleus having linked directly thereto a radical of the formula:



wherein Z is a lower alkylene radical and X is a dihydroxyphenyl silver halide developing radical, said



substituents containing the only silver halide developing radical in said dye developer, providing as a function of the development an image-wise distribution of unoxidized dye developer in undeveloped areas of said emulsion, and transferring at least part of said distribution of said unoxidized dye developer by imbibition from said emulsion to an image-receiving layer in superposed relationship with said emulsion to impart to said image-receiving layer a positive dye image.

2. A process as defined in claim 1 wherein said aqueous alkaline solution also contains an auxiliary silver halide developer.

3. A process as defined in claim 1 wherein said dye developer is disposed prior to exposure in a photosensitive element comprising said silver halide emulsion, the anthraquinone nucleus of said dye developer being in its leuco form and subsequent to exposure oxidizing said leuco form to the anthraquinone form.

4. A process as defined in claim 1 wherein there are two  $-\text{NH}-\text{Z}-\text{X}$  radicals present in said dye developer and said  $-\text{NH}-\text{Z}-\text{X}$  radicals are substituted in the 1 and 4 positions of the anthraquinone nucleus.

5. A process as defined in claim 4 wherein X is a para-dihydroxyphenyl silver halide developing radical.

6. A process as defined in claim 4 wherein X is an ortho-dihydroxyphenyl silver halide developing radical.

7. A process as defined in claim 1 wherein there is one  $-\text{NH}-\text{Z}-\text{X}$  radical present in said dye developer said  $-\text{NH}-\text{Z}-\text{X}$  radical being substituted in the 1 position of the anthraquinone nucleus and the 4 position of said anthraquinone nucleus being substituted by an alkyl amino group.

8. A process as defined in claim 7 wherein the alkyl group of said alkyl amino group is a hydroxy alkyl radical.

9. A process as defined in claim 8 wherein said hydroxy alkyl group is a hydroxy secondary alkyl group and the secondary carbon atom of said hydroxy secondary alkyl group is attached to the amino group.

10. A process as defined in claim 7 wherein X is a para-dihydroxyphenyl silver halide developing radical and the alkyl group of said alkyl amino group comprises less than 6 carbon atoms.

11. A process as defined in claim 7 wherein X is an ortho-dihydroxyphenyl silver halide developing radical and the alkyl group of said alkyl amino comprises less than 6 carbon atoms.

12. A process as defined in claim 1 wherein said dye developer is 1,4 - bis - ( $\alpha$ -methyl- $\beta$ -hydroquinonyl-ethylamino)-anthraquinone.

13. A process as defined in claim 1 wherein said dye developer is 1,4 - bis( $\alpha$  - methyl- $\beta$ -hydroquinonyl-ethylamino)-5,8-dihydroxyanthraquinone.

14. A process as defined in claim 1 wherein said dye developer is 1 - ( $\alpha$  - hydroxymethyl-propylamino)-4-( $\alpha$ -methyl- $\beta$ -hydroquinonyl-ethylamino)-anthraquinone.

15. A process as defined in claim 1 wherein said dye developer is 1 - ( $\alpha$  - hydroxymethyl-propylamino)-4-( $\alpha$ -methyl -  $\beta$  - hydroquinonyl-ethylamino) - 5,8-dihydroxyanthraquinone.

16. A process as defined in claim 1 wherein said dye developer is 1,4 - bis( $\alpha$  - methyl- $\beta$ -hydroquinonyl-ethylamino)-5,8-bis-benzenesulfonamido-anthraquinone.

17. In a photographic product comprising a photosensitive element, an image-receiving layer and a rupturable container holding an aqueous alkaline processing solution, said photosensitive element being adapted so as to be capable of being superposed on the image-receiving layer and said rupturable container being adapted so as to be capable of being ruptured and dispensing the aqueous alkaline processing solution between said superposed photosensitive element and said image-receiving layer, the feature of disposing in said photosensitive element a dye developer having an anthraquinone nucleus, at least one and not more than two of the nuclear carbon atoms of said anthraquinone nucleus having linked directly thereto a radical of the formula:



wherein Z is a lower alkylene radical and X is a dihydroxyphenyl silver halide developing radical, said



substituents containing the only silver halide developing radical in said dye developer.

18. A photographic product as defined in claim 17 wherein there are two  $-\text{NH}-\text{Z}-\text{X}$  radicals present in said dye developer and said  $-\text{NH}-\text{Z}-\text{X}$  radicals are

21

substituted in the 1 and 4 positions of said anthraquinone nucleus.

19. A process of developing an exposed photosensitive silver halide emulsion which comprises developing an exposed silver halide emulsion with an aqueous alkaline processing solution containing a dye developer having an anthraquinone nucleus, at least one and not more than two of the nuclear carbon atoms of said anthraquinone nucleus having linked directly thereto a radical of the formula:



wherein Z is a lower alkylene radical and X is a dihydroxyphenyl silver halide developing radical, said



substituents containing the only silver halide developing radical in said dye developer.

20. A process as defined in claim 19 wherein said aqueous alkaline processing solution also contains an auxiliary silver halide developer.

21. A process as defined in claim 19 wherein there are two  $-\text{NH}-\text{Z}-\text{X}$  radicals present in said dye developer and said  $-\text{NH}-\text{Z}-\text{X}$  radicals are substituted in the 1 and 4 positions of the anthraquinone nucleus.

22. A process as defined in claim 19 wherein X is a para-dihydroxyphenyl silver halide developing radical.

23. A process as defined in claim 19 wherein X is a ortho-dihydroxyphenyl silver halide developing radical.

24. A process as defined in claim 19 wherein there is one  $-\text{NH}-\text{Z}-\text{X}$  radical present in the dye developer, said  $-\text{NH}-\text{Z}-\text{X}$  radical being substituted in the 1 position of the anthraquinone nucleus and the 4 position of said anthraquinone nucleus is substituted by an alkyl amino group.

25. A process as defined in claim 24 wherein the alkyl group of said alkyl amino group is a hydroxy alkyl radical.

26. A process as defined in claim 25 wherein said hydroxy alkyl group is a hydroxy secondary alkyl group and the secondary carbon atom of said hydroxy secondary alkyl group is attached to the amino group.

27. A process as defined in claim 24 wherein X is a para-dihydroxyphenyl silver halide developing radical and the alkyl group of said alkyl amino group comprises less than 6 carbon atoms.

28. A process as defined in claim 24 wherein X is an ortho-dihydroxyphenyl silver halide developing radical and the alkyl group of said alkyl amino group comprises less than 6 carbon atoms.

29. A photographic product comprising a plurality of layers including a silver halide emulsion layer, a layer contiguous with said silver halide emulsion layer containing a dye developer having an anthraquinone nucleus, at least one and not more than two of the nuclear carbon atoms of said anthraquinone nucleus being joined to a radical represented by the formula:



wherein Z is a lower alkylene radical and X is a dihydroxyphenyl silver halide developing radical, said  $-\text{NH}-\text{Z}-\text{X}$

22

substituents containing the only silver halide developing radical in said dye developer.

30. A photographic product as defined in claim 29 wherein there are two  $-\text{NH}-\text{Z}-\text{X}$  radicals present in said dye developer, said  $-\text{NH}-\text{Z}-\text{X}$  radicals are substituted in the 1 and 4 positions of the anthraquinone nucleus and X is a para-dihydroxyphenyl silver halide developing radical.

31. A photographic product as defined in claim 29 wherein there are two  $-\text{NH}-\text{Z}-\text{X}$  radicals present in said dye developer, said  $-\text{NH}-\text{Z}-\text{X}$  radicals are substituted in the 1 and 4 positions of the anthraquinone nucleus and X is an ortho-dihydroxyphenyl silver halide developing radical.

32. A photographic product as defined in claim 29 wherein there is one  $-\text{NH}-\text{Z}-\text{X}$  radical present in said dye developer, said  $-\text{NH}-\text{Z}-\text{X}$  radical is substituted in the 1 position of the anthraquinone nucleus, the 4 position of said anthraquinone nucleus being substituted by an alkyl amino group, said X being a para-dihydroxyphenyl silver halide developing radical and the alkyl group of said alkyl amino group in the 4 position comprising less than 6 carbon atoms.

33. A photographic product as defined in claim 29 wherein there is one  $-\text{NH}-\text{Z}-\text{X}$  radical present in said dye developer, said  $-\text{NH}-\text{Z}-\text{X}$  radical is substituted in the 1 position of the anthraquinone nucleus and the 4 position of said anthraquinone nucleus is substituted by an alkyl amino group, said X radical being an ortho-dihydroxyphenyl silver halide developing radical and the alkyl portion of said alkyl amino group comprising less than 6 carbon atoms.

34. A product as defined in claim 29 wherein said dye developer is 1,4-bis-( $\alpha$ -methyl- $\beta$ -hydroquinonyl - ethylamino)-anthraquinone.

35. A product as defined in claim 29 wherein said dye developer is 1,4-bis-( $\alpha$ -methyl- $\beta$ -hydroquinonyl - ethylamino)-5,8-dihydroxyanthraquinone.

36. A product as defined in claim 29 wherein said dye developer is 1-( $\alpha$ -hydroxymethyl-propylamino) - 4 - ( $\alpha$ -methyl- $\beta$ -hydroquinonyl-ethylamino)-anthraquinone.

37. A product as defined in claim 29 wherein said dye developer is 1-( $\alpha$ -hydroxymethyl-propylamino) - 4 - ( $\alpha$ -methyl- $\beta$ -hydroquinonyl-ethylamino) - 5,8 - dihydroxyanthraquinone.

38. A product as defined in claim 29 wherein said dye developer is 1,4-bis-( $\alpha$ -methyl- $\beta$ -hydroquinonyl - ethylamino)-5,8-bis-benzensulfonamido)anthraquinone.

#### References Cited in the file of this patent

#### UNITED STATES PATENTS

2,983,600 Rogers ----- May 9, 1961

#### FOREIGN PATENTS

682,665 Great Britain ----- Nov. 12, 1952

#### OTHER REFERENCES

Venekataraman Synthetic Dyes, vol. 1, Academic Press, N.Y. (1952), pp. 358-9.

UNITED STATES PATENT OFFICE  
CERTIFICATE OF CORRECTION

June 2, 1964

Patent No. 3,135,606

Elkan R. Blout et al.

It is hereby certified that error appears in the above numbered patent requiring correction and that the said Letters Patent should read as corrected below.

Column 2, lines 69 and 70, for "prefered" read -- preferred  
--; column 5, line 17, for "anthraquinione" read -- anthraquinone  
--; column 7, line 66, for "anthraquionne" read -- anthraquinone  
--; column 8, line 35, for "2-beta-" read -- 2-(beta- --;  
column 10, line 2, for "to" read -- into --; line 46, for  
"monoethyl" read -- monomethyl --; column 11, lines 28 and 29,  
for "monoethyl" read -- monomethyl --; column 13, line 1, for  
"O-" read -- ~~β~~--; column 18, line 48, after "dye" insert  
-- developer --; column 20, line 34, after "amino" insert  
-- group --; line 40, for "-bis(α-)" read -- -bis-(α- --; line  
50, for "-bis(α-)" read -- -bis-(α- --; same column 20, line  
62, for "antharaquinone" read -- anthraquinone --; column 21,  
line 27, for "a" read -- an --; line 49, for "carobn" read  
-- carbon --; column 22, line 48, for "-benzensulfonamido)-  
anthraquinone" read -- benzenesulfonamido-anthraquinone --;  
line 52, for "2,983,600" read -- 2,983,606 --; line 58, for  
"Venekataraman" read -- Venkataraman --.

Signed and sealed this 3rd day of November 1964.

(SEAL)

Attest:

ERNEST W. SWIDER  
Attesting Officer

EDWARD J. BRENNER  
Commissioner of Patents